# EUROPEAN PATENT SPECIFICATION

(11) **EP 0 191 008 B1**
(45) Date of publication and mention of the grant of the patent: **15.03.1989**
(21) Application number: 86850030.7
(22) Date of filing: 31.01.1986
(51) Int. Cl.: B22D 23/00

(54) **Shell or tubular object and method to manufacture the same**
Hülsen- oder rohrförmiger Gegenstand und Verfahren zu seiner Herstellung
Carapace ou objet tubulaire et leur procédé de fabrication

(30) Priority: 01.02.1985 SE 8500473
(43) Date of publication of application: 13.08.1986
(73) Proprietor: AB VOLVO, 405 08 Göteborg (SE)
(72) Inventor: Björklund, Nils-Eric, S-73400 Hallstahammar (SE); Lindgren, Hâkan, S-73400 Hallstahammar (SE); Gustafson, Sten, S-72211 Västerâs (SE); Dahlén, Mats, S-41652 Göteborg (SE)
(74) Representative: Säfwenberg, Björn

(56) References cited:
- FR-A- 2 431 335
- PATENTS ABSTRACTS OF JAPAN, vol. 8, no. 67 (C-216) [1504], 29th March 1984; & JP - A - 58 217 671 (MITSUBISHI JUKOGYO K.K.) 17-12-1983
- PATENTS ABSTRACTS OF JAPAN, vol. 7, no. 46 (C-153) [1191], 23rd February 1983; & JP - A - 57 198 256 (ISUZU JIDOSHA K.K.) 04-12-1982

## Description

The invention relates to a method to manufacture a shell or tubular object to be incorporated in a heat and corrosion resistant part of a combustion engine, as defined in the first part of claim 1.

The background of the invention is a desire to make it possible to operate internal combustion engines at a higherworking temperature, whereby an increased efficiency and a more complete combustion can be achieved. Thus, it is a well-known problem to accomplish temperature and corrosion resistance of the materials, especially in combustion chambers and exhaust channels, in case the working temperature is to be raised above what is normal in today's engines.

In fact, ceramic materials are high-temperature and corrosion resistant, but it is complicated and expensive to combine ceramics with other, metallic construction materials, such as iron and nickel alloys. Tensions are caused by different temperature coefficients. Certain ceramics will also be subjected to phase transformations in temperature intervals within or very close to the working temperatures in question. Moreover, the subsequent treatment, e. g. the boring of holes, becomes more difficult, if ceramics are used.

Furthermore, experiments have been made to coat especially exposed motor parts with plates or surface layers of some kind of heat and corrosion resistant metal alloy, e. g. of a FeCrAI- type, which however causes problems in case inside cavities, in particular of a complicated geometry, are to be coated.

It has also been suggested (FR-A-2 431 335) to manufacture tubular surface bodies, which have been thermally sprayed in advance, with a remaining mandrel or core. In using this known method, however, only very simple, especially cylindrical or conical tube forms can be used, since it must be possible to take out the mandrel or core after molding.

Furthermore, the published Swedish Patent Application SE-A-8 300 603-1 discloses a method of manufacturing a machine part, including a heat insulated inlet gas channel, by thermally spraying a very thin first layer, having a thickness of 0.1-0.2 mm, of a soft metal material, such as zinc, tin, lead, copper or aluminium, onto a sand core. A second layer, having a thickness of 0.5-2.5 mm, of a metal material, such as carbon steel, is thermally sprayed onto the first layer, and thereafter a third layer, serving as a heat barrier and consisting of a ceramic material is applied, e. g. by thermal spraying. Then, the sand core with the three layers applied thereon is placed in a mold for molding the machine part in a conventional manner. Upon molding, the sand core is removed, so that the three layers form an internal surface of a channel in the machine part.

However, in this known methods, there might be a risk of cracking when thermally spraying the various layers having different expansion characteristics. Futhermore in the method disclosed by SE-A-8 300 603-1, the innermost layer, forming the internal surface layer of the machine part, is not corrosion resistant and is not suitable e. g. for exhaust channels. Also, the melting point of the soft metal material is far too low to permit the use in an exhaust channel of a combustion engine. Thus, a typical temperature of the exhaust gases is about 850 °C, whereas the melting point of Zn is about 420 °C.

The object of the invention is to eliminate the disadvantages and restrictions of the known methods and to enable a simple manufacture of shell or tubular objects, even with a complicated geometry, by thermal spraying of a heat and corrosion resistant metal alloy so as to form a dense, first surface layer and an additional layer serving as a heat barrier, without any risk of cracking during the spraying process. A further object is to enable the molding of such an object into a molded body having one or several channels or cavities constituted by the molded shell or tubular object according to the invention.

The main object is achieved by a method as defined in the characterizing clause of claim 1. The invention also relates to a shell or tubular object to be incorporated in a machine part of a combustion engine, as defined in claim 6. Other suitable features are stated in the claims 2-5 and 7, respectively.

Thus, when manufacturing such an object it is essential that the core body, onto which a first layer is sprayed, will be removed before additional material is applied by spraying. It is particularly suitable to make the core body of molding sand which can loose its form stability and be discharged from the tube or shell, e. g. upon heating. Without risk of cracking due to tensions, which would unavoidably arise if the core body were to remain, continuous spraying may thereafter be effected up to a desired thickness.

The thermal spraying of the additional layer should be controlled in such a way that the second or third layer contains more oxides and/or pores than the first layer, whereby the desired qualities, especially a lower thermal conductivity, are obtained in the second or third layer. Naturally, it is also possible to apply a relatively thin layer, either as a second layer between a first and a third layer or as a third layer sprayed onto the second layer. Preferably, such a relatively thin layer may e. g. be used as a diffusion barrier for carbon or nickel. Also, it can be used to increase the mechanical qualities at higher temperatures.

The invention will be explained further below with reference to the appended drawings illustrating an embodiment.
Fig. 1 shows schematically a sand core ;
Fig. 2 shows said sand core with a first layer sprayed thereupon ;
Fig. shows the desired tubular object after removing the sand core and spraying a relatively thick second layer onto the first layer.

Thus, in a way known per se, a core body 1 is made of molding sand and a phenol resin as a binding agent. As shown in Fig. 1, the core body 1 has an external configuration of the tubular object and, in addition thereto, holding portions 1a, 1b at each end for holding the core body. In the embodiment, the desired object comprises an exhaust channel in a cylinder head of a combustion engine.

In accordance with Fig. 2, a relatively thin and essentially pore-free layer 2 of a metal alloy containing about 5 % Al, 22 % Cr and the rest mainly Fe (the contents are by weight) is sprayed onto the core body 1. Porosity, if any, must consist of closed pores. When the layer thickness is at least 0.5 mm, preferably about 1 mm, the spraying operation is interrupted, whereupon the sand core 1 is removed in that the sand core and the layer sprayed thereon is heated in a furnace at about 600 °C for 2-3 hours, and thereafter the sand is discharged from the tubular metal alloy layer 2.

Thereafter, a second layer 3 is sprayed onto the first, self-supporting layer 2. In absence of a core body, the first layer is permitted to expand and shrink freely due to variations of temperature, without any risk of tensions and accompanying cracking. The thickness of the second layer may be at least 1 mm. The spraying process can be performed without interruption for cooling.

Different methods of spraying are possible. Preferably, the first, relatively thin layer 2 is sprayed by means of a wire-fed flame sprayer so as to form a dense layer. In case a surface layer of great purity is desired (small quantities of oxides and pores), the layer may be applied by plasma spraying. The second layer 3 may preferably be applied by means of a powder-fed flame sprayer in order to obtain a suitable quantity of pores and oxides. In this case, a quantity of 5-25 %, preferably about 15 %, pores and oxides is desired. However, the second layer 3 does not have to be of the same material composition as the first layer 2, but may e. g. consist of another metal alloy of high heat resistance.

With regard to the heat tensions which may appear in the material, it is certainly an advantage if the layer consists of the same material and differs only in porosity and oxide contents. Moreover, a thin third layer may be applied either between or on top of the two above-mentioned layers. The third layer may i. a. function as an adhesive layer or diffusion barrier.

The object and the manufacturing method according to the invention have several advantages. The geometric shape as well as the materials and the thickness thereof can be chosen at will. Thus, very thick layers (the second layer 3) may be applied after the removal of the core body. Moreover, the manufacturing method is relatively quick (metal can be sprayed onto a red hot substrate) and the handling rather simple. The cassation is very low because of the eliminated risk of cracking. Even the subsequent operations, e. g. molding, are facilitated and can therefore be performed with great accuracy. Moreover, by avoiding ceramic materials, the recircling of scrap is made easier.

## Claims

1. A method to manufacture a shell or tubular object to be incorporated in a heat and corrosion resistant part of a combustion engine, said object being manufactured by thermal spraying of a first layer (2) of a high temperature resistant metal alloy material onto a core body (1), the external dimensions of which correspond to the internal dimensions of the finished object, characterized in that after the first, dense layer (2) is formed by thermal spraying of a high temperature and corrosion resistant metal alloy material onto said core body (1), the core body (1) is removed so as to leave a self-supporting shelle or tube, and at least one additional layer (3) is formed by thermal spraying of a heat resistant metal alloy material onto the external surface of said self-supporting shell or tube (2), one such additional layer (3) being applied to a greater thickness than said first layer (2) and the thermal spraying being controlled in such a way that said additional layer (3) contains more oxides and/or pores than the first layer (2) and serves as a heat barrier in the finished object (2, 3).

2. A method according to claim 1, characterized in that the core body (1) is made of molding sand.

3. A method according to claim 1 or 2, characterized in that the material being used when spraying said first layer (2) consists of 1-12 % Al, 10-30 % Cr, possibly small quantities of one or several elements of the group Si, Mn, Co, Y, Hf, possibly small quantities of oxides and nitrides and the rest Fe.

4. A method according to any one of claims 1-3, characterized in that the same material is used when spraying said first layer (2) and said at least one additional layer (3).

5. A method according to any one of claims 1-4, characterized in that said at least one additional layer includes a second layer and a third layer, said second or third layer being substantially thinner than the other two layers and serving as an adhesive layer or a diffusion barrier.

6. A shell or tubular object, obtainable by the method defined in any one of claims 1-5, to be incorporated in a part of a combustion engine, said object having at least two layers (2, 3) of a high temperature resistant metal alloy material, characterized in that the first, dense, thermally sprayed layer (2) has a thickness of 0.5-1.5 mm and that the porosity of the first layer (2) consists of closed pores, whereas the total porosity and oxide contents of an additional third layer (3) exceeds 10 %, said additional third layer (3) serving as heat barrier.

7. An object according to claim 6, characterized in that a second or third layer (3) has a thickness greater than 1 mm, preferably about 2.5 mm.

## Patentansprüche

1. Ein Verfahren zur Herstellung eines hülsen-oder rohrförmigen Gegenstandes, der in einen hitze- und korrosionsbeständigen Teil eines Verbrennungsmotors eingebaut werden soll, wobei der Gegenstand durch thermisches Aufsprühen einer ersten Schicht (2) aus einem hochtemperaturbeständigen Metall-Legierungsmaterial auf einen Kernkörper (1) hergestellt wird, dessen Außenabmessungen den Innenabmessungen des fertigen Gegenstandes entsprechen, dadurch gekennzeichnet, daß, nachdem die erste, dichte Schicht (2) durch thermisches Aufsprühen eines hochtemperatur- und korrosionsbeständigen Metall-Legierungsmaterials auf den Kernkörper (1) gebildet ist, der Kernkörper (1) entfernt wird, so daß eine selbsttragende Hülse oder ein selbsttragendes Rohr verbleibt, und daß durch thermisches Aufsprühen eines hitzebeständigen Metall-Legierungsmaterials auf die Außenfläche der selbsttragenden Hülse oder des selbsttragenden Rohres (2) wenigstens eine zusätzliche Schicht (3) gebildet wird, wobei eine solche zusätzliche Schicht (3) mit größerer Dicke als die erste Schicht (2) aufgebracht und das thermische Aufsprühen derart gesteuert wird, daß die zusätzliche Schicht (3) mehr Oxide und/oder Poren als die erste Schicht (2) enthält und als Hitzesperre im fertigen Gegenstand (2, 3) dient.

2. Ein Verfahren nach Anspruch 1, dadurch gekennzeichnet, daß der Kernkörper (1) aus Formsand gemacht wird.

3. Ein Verfahren nach Anspruch 1 oder 2, dadurch gekennzeichnet, daß das Material, welches beim Aufsprühen der ersten Schicht (2) verwendet wird, aus 1 bis 12 % AI, 10 bis 30 % Cr, gegebenenfalls kleinen Mengen an einem oder mehreren Elementen der Gruppe Si, Mn, Co, Y, Hf, gegebenenfalls kleinen Mengen an Oxiden und Nitriden und der Rest aus Fe besteht.

4. Ein Verfahren nach einem der Ansprüche 1 bis 3, dadurch gekennzeichnet, daß beim Aufsprühen der ersten Schicht (2) und der wenigstens einen zusätzlichen Schicht (3) dasselbe Material verwendet wird.

5. Ein Verfahren nach einem der Ansprüche 1 bis 4, dadurch gekennzeichnet, daß die wenigstens eine zusätzliche Schicht eine zweite Schicht und eine dritte Schicht einschließt, wobei die zweite oder dritte Schicht im wesentlichen dünner als die beiden anderen Schichten sind und als eine Adhäsionsschicht oder eine Diffusionssperre dienen.

6. Ein hülsen- oder rohrförmiger Gegenstand, herstellbar durch das Verfahren nach einem der Ansprüche 1 bis 5 zum Einbau in einen Teil eines Verbrennungsmotors, wobei der Gegenstand wenigstens zwei Schichten (2, 3) aus einem hochtemperaturbeständigen Metall-Legierungsmaterial hat, dadurch gekennzeichnet, daß die erste, dichte, thermisch aufgesprühte Schicht (2) eine Dicke von 0,5 bis 1,5 mm hat und daß die Porosität der ersten Schicht (2) aus geschlossenen Poren besteht, während die Gesamtporosität und die Oxidgehalte einer zusätzlichen dritten Schicht (3) 10 % überschreiten, wobei die zusätzliche dritte Schicht (3) als Hitzesperre dient.

7. Ein Gegenstand nach Anspruch 6, dadurch gekennzeichnet, daß eine zweite oder dritte Schicht (3) eine Dicke größer als 1 mm, vorzugsweise eine Dicke von etwa 2,5 mm haben.

## Revendications

1. Procédé de fabrication d'un objet en coque ou tubulaire à incorporer dans une pièce résistant à la chaleur et à la corrosion de moteur à combustion, ledit objet étant fabriqué par projection à chaud d'une première couche (2) d'un matériau du type alliage métallique résistant aux hautes températures sur un corps de noyau (1), à dimensions extérieures correspondant aux dimensions intérieures de l'objet fini, caractérisé en ce qu'après avoir constitué la première couche dense (2) par projection à chaud d'un matériau du type alliage métallique résistant aux hautes températures et à la corrosion sur ledit corps de noyau (1), on élimine le corps de noyau (1) de façon à laisser subsister une coque ou un tube auto-portant, et l'on forme au moins une couche additionnelle (3) par projection à chaud d'un alliage métallique résistant à, la chaleur sur la surface extérieure de ladite coque ou dudit tube auto-portant (2), une telle couche additionnelle (3) étant appliquée sur une plus grande épaisseur que ladite première couche (2) et la projection à chaud étant réglée en sorte que ladite couche additionnelle (3) contienne davantage d'oxydes et/ou de pores que la première couche (2) et serve de barrage thermique dans l'objet fini (2, 3).

2. Procédé selon ia revendication 1, caractérisé en ce que le corps de noyau (1) est en sable de moulage.

3. Procédé selon la revendication 1 ou 2, caractérisé en ce que le matériau utilisé lors de la projection de ladite première couche (2) est composé de 1 à 12% d'AI, 10 à 30% de Cr, éventuellement de petites quantités d'un ou plusieurs éléments du groupe Si, Mn, Co, Y, Hf, éventuellement de faibles quantités d'oxydes et de nitrures et pour le reste de Fe.

4. Procédé selon l'une quelconque des revendications 1 à 3, caractérisé en ce qu'on utilise le même matériau lors de la projection de ladite première couche (2) et de la ou de chaque susdite couche additionnelle (3).

5. Procédé selon l'une quelconque des revendications 1 à 4, caractérisé en ce que la ou chaque susdite couche additionnelle comporte une seconde couche et une troisième couche, ladite seconde ou troisième couche étant sensiblement plus mince que les deux autres couches et servant de couche adhésive ou de barrage à la diffusion.

6. Objet en coque ou tubulaire, pouvant être obtenu par le procédé défini dans l'une quelconque des revendications 1 à 5, à incorporer dans une pièce de moteur à combustion, ledit objet comportant au moins deux couches (2, 3) d'un matériau du type alliage métallique résistant aux hautes températures, caractérisé en ce que la première couche dense (2) projetée à chaud a une épaisseur de 0,5 à 1,5 mm et que les pores de la première couche (2) sont des pores fermés, tandis que les teneurs totales en pores et en oxydes d'une troisième couche additionnelle (3) dépasse 10 %, ladite troisième couche additionnelle (3) servant de barrage thermique.

7. Objet selon la revendication 6, caractérisé en ce qu'une seconde ou troisième couche (3) a une épaisseur supérieure à 1 mm, de préférence d'environ 2,5 mm.
